

Patented Feb. 22, 1938

2,108,837

# UNITED STATES PATENT OFFICE

2,108,837

## TEXTILE MATERIAL CONTAINING ORGANIC ESTERS OF CELLULOSE AND METHOD OF PREPARING SAME

William Whitehead, Cumberland, Md., assignor  
to Celanese Corporation of America, a corpora-  
tion of Delaware

No Drawing. Application April 3, 1935,  
Serial No. 14,472

12 Claims. (Cl. 8—20)

This invention relates to the preparation and manufacture of yarns, filaments, fabrics and other articles from organic esters of cellulose, which organic esters have been subjected at least 5 in part to the action of a saponifying agent and relates more particularly to the preparation of the yarns and filaments of organic esters of cellulose prior to the application thereto of a basic material for the purpose of saponifying same or 10 sensitizing same for subsequent saponification.

An object of the invention is the economic and expeditious production of textile materials containing yarns and filaments of an organic esters of cellulose, at least a part of said mate- 15 rials having been treated with a saponifying agent. A further object of this invention is the partial and intermittent saponification of yarns during a winding operation and the preparation of such yarns, so that they will evenly and quickly 20 react to the saponifying material and/or permit the saponifying material to quickly penetrate into the filaments immediately upon contact therewith and to an extent sufficient to use up substantially all the saponifying material or at 25 least carry it into the filaments prior to being wound upon the take-up package so that blurring or streaky saponification is prevented. Other objects of the invention will appear from the following detailed description.

I have found that the speed with which a saponifying agent reacts with or is caused to penetrate into a yarn containing organic esters of cellulose is proportionate to the amount of moisture contained in the filaments of the yarn 30 and also that the depth and evenness of the saponifying action is proportionate to the amount of moisture contained in the filaments of the yarn. By employing this invention, which, in general, consists in conditioning the yarn prior to treatment with a saponifying agent such that it 35 contains substantially its maximum content of moisture regain, there may be employed less saponifying material, which reduction in saponifying material also produces a reduction in the 40 amount of crystals of salt formed on the yarn. By thus reducing the amount of crystals at the 45 places saponified the yarn becomes more amenable to textile operations. By employing this invention yarns may be sufficiently saponified during 50 the winding operation so that they become sensitized for further and heavy saponification in soap baths without producing on the yarn a sufficient amount of crystalline material to inter- 55 fere with the same as the yarns are passed

through guides, needles, etc., in the future processing operations.

By employing this invention the saponification of the yarns during the winding operation is caused to go to completion very rapidly. In this 5 manner when periodically or intermittently saponifying yarns there is developed a very sharp line between the part saponified and the untreated part as the action of saponification and the penetration of the saponifying agent is so rapid 10 that the tendency of the saponifying medium to travel along the yarn is prevented as the same is used up prior to any substantial lengthwise movement thereof.

By employing this invention there may be pre- 15 vented any action of the saponifying agent upon the uncontacted area of the yarn. In prior meth- 20 ods of intermittently or periodically saponifying yarns during a winding operation the action of the saponifying agent was not carried sufficiently 25 toward completion prior to winding of the yarn upon the take-up package, thus producing an action on the uncontacted part of the yarn where the contacted part of the yarn crossed same in the package. Although the action of the 30 saponifying agent after it had reached the take- 35 up package was slight, in future treatments and development of the yarn by treatment in a soap bath these places receiving slight actions were amplified to such an extent that in a dyed mate- 40 rial a smudge or blur was produced. By employing this invention very strong concentrations of 45 saponifying agents may be placed on the yarn during the winding operation, yet the same is sufficiently reacted or carried to the interior of the filaments so that there is substantially no transfer of unreacted saponifying agents from the treated portion of the yarn to the untreated 50 portion of the yarn on the take-up package. This gives rise to clear cut lines between the treated 55 and the untreated part of the yarn.

By employing this invention a still further ad- 55 vantage is obtained in that the saponified yarn produced is more evenly saponified. In plac- 60 ing a saponifying medium upon a yarn by means of a furnishing device during a winding opera- 65 tion, it is very difficult to contact all parts of the yarn with an even amount of saponifying mate- 70 rial. However, by employing this invention the evenness of application is compensated for by the 75 affinity of the yarn for the saponifying agent which results in an even saponification. Al- 80 though any unevenness in saponification is slight during this operation if the material is later treated in a soap solution and then dyed any 85

unevenness is greatly magnified and becomes very obvious. By employing this invention fabrics may be further developed by treatment in soap baths and the like and then dyed which do not 5 show an unevenness of saponification.

In accordance with my invention then I partially and lightly saponify yarns and filaments containing organic esters of cellulose, which 10 yarns contain substantially a maximum amount of moisture regain to sensitize the same, which sensitizing may cover the entire yarn or filament or may be applied thereto intermittently, periodically or at random, and then either before or 15 after forming the yarns and filaments into fabrics I treat the same in a bath having a pH value from 8 to 11 or more for the purpose of developing or further saponifying the yarn or only that part of the yarn which has been sensitized. Also, 20 in accordance with my invention, I treat yarns and filaments or textile materials such as warps or fabric containing organic esters of cellulose by placing same in a humid atmosphere having a fairly high relative humidity so that the yarns, etc. will regain a substantial amount of moisture 25 and then treat these yarns with a basic material, for instance, with the aid of a printing device, for the purpose of saponifying them or sensitizing the same for saponification.

This invention is applicable to the treatment 30 of yarns or filaments or fabrics of any suitable ester of cellulose that is capable of being partially and/or totally saponified by treatment with bases. For example, I may employ this invention in the treatment of yarns and filaments 35 and fabrics formed from the nitrates of cellulose or the organic esters of cellulose or mixture of same. Examples of organic esters of cellulose are cellulose acetate, cellulose propionate and cellulose butyrate. The yarns or filaments containing 40 these materials may be formed by either the wet or dry method of spinning and may contain besides the derivatives of cellulose, dyes, lakes, fillers, plasticizers and lubricants.

Yarns and filaments or textile materials 45 formed of the esters of cellulose may contain up to 5.5% or more, on their weight, of moisture depending upon the humidity of the atmosphere in which they are placed. These materials regain a moisture content corresponding to the rise in 50 relative humidity of the atmosphere in which they are placed. For instance, cellulose acetate which has been stored for a period of time may drop in moisture content such that the moisture content is below 1 per cent. However, when 55 placed in an atmosphere containing a relative humidity of 65% or above, the yarns and filaments will regain a moisture content of up to 5.5 or more of their weight. The speed of action and penetration of any saponifying agent applied 60 to the yarns will be proportionate to the amount of moisture that the yarn has regained prior to contact with the saponifying agent even though the saponifying agent be applied to the yarns from an aqueous solution. Thus, for producing sharp lines of saponification and an even 65 saponifying action, it is preferable to have this moisture regain or content of the yarn as near the maximum as possible.

70 For the purpose of producing substantially the maximum moisture regain in the yarn or fabric prior to contacting same with a saponifying agent, the yarn may be stored immediately prior to contacting with the saponifying agent in a 75 chamber or container, the atmosphere of which

is kept fairly saturated with moisture, that is, for instance, an atmosphere having a relative humidity of above 40 per cent. Further, the yarn may be made more susceptible to the action of the saponifying agent at the winding operation 5 by placing the feed bobbin on the winding machine in a humidor having a fairly high humidity, for instance, about 85 per cent relative humidity. A still further method of building up the moisture regain of the yarn is to surround the twisting machine, or at least that part of it traversed by the yarn, by an atmosphere that has a relatively high humidity, for instance, about 65 per cent relative humidity. The maintaining of the atmosphere, through which the yarn passes during the winding operation, at a high percentage of relative humidity is of advantage even when the yarn has been previously conditioned or when it is fed from a humidor. The atmosphere may be kept at a high humidity by the escaping of steam near the feed of the yarn or by suitable humidifiers employing atomized water, placed near the machine. Any other suitable method or device may be employed for supplying the yarn with sufficient moisture that the moisture regain 25 or moisture absorbed by the yarn is approximately that of the maximum moisture content that the yarn will pick up.

This invention is particularly applicable to the treatment of yarns or fabrics with a saponifying 30 agent during a winding operation, for instance, by contacting the yarns with a furnishing device supplying thereto a solution of a basic material capable of producing at least sufficient saponification to etch the surface of the yarn. Thus, 35 after the yarns have been conditioned, by raising their moisture content, and made susceptible to the saponifying action they may be caused to pass over a wick or roller that dips into a solution containing a base material. The yarns may be 40 caused to contact the wick or roller continuously or periodically to produce yarns which are lightly saponified or sensitized throughout their length or only at certain periods of their length. For 45 fabrics this can be done on any suitable device, for instance, on a printing machine. When treating fabrics the fabric may be conditioned by storage in a moist atmosphere and/or unrolled from a suitable humidor.

The saponifying agent applied to the yarns or 50 fabrics during the winding operation need only be sufficient to etch the yarns as the heavy or substantial part of the saponification can be later developed by treating the yarns or fabrics in a soap solution or other bath having a relatively 55 mild saponifying action, or one that would not normally saponify the material at all. The developing bath produces a saponification of the material at the parts sensitized during the winding operation and has substantially no effect upon 60 that part of the yarn or fabric not contacted with the saponifying material during the winding operation. The action of applying a saponifying agent to the material during a winding operation such that there is a partial saponification of the 65 yarn or fabric to an extent that the loss in weight of the yarn at those points contacted is from 2 to 7 per cent of their weight may be termed a sensitizing action.

The sensitizing material may be any suitable 70 basic material or a solution of a base material having a pH value of from 10 to 14. Any suitable basic solution may be employed for this purpose such as an aqueous solution or an alcoholic solution of an alkali hydroxide, for in- 75

stance, sodium hydroxide or potassium hydroxide, an aqueous solution of ammonium hydroxide, a salt of a strong base such as ammonia or alkali and a weak acid such as the organic acids, organic compounds having a basic reaction, etc. Examples of salts of a strong base and an organic acid which may be employed for this invention are sodium acetate, potassium acetate, etc. Examples of organic bases that may be employed as the sensitizing agent are the primary, secondary and tertiary amines, for instance, ethanol amine, methanol amine, di-methanol amine, di-ethanol amine, tri-methanol amine and tri-ethanol amine. Also, the quaternary ammonium bases may be employed, for instance, tetramethyl ammonium hydroxide, tetraethyl ammonium hydroxide, etc.

These materials may be applied to the yarn from aqueous solutions which solutions may be of any suitable concentration such as the pH value of the solution has a value of above 10. In the treatment of yarns which are to be used in certain types of machines wherein they of necessity must pass through small guide eyes and needles, it is sometimes advisable to select a sensitizing agent which, when applied to the yarn and after reaction with the acid radicle thereof, forms a salt, the crystals of which do not interfere as the yarn passes through said guides. The length of treatment that the materials receive in such solutions is preferably limited such that the materials are not saponified to any great extent. For instance, it is found preferable in most cases to limit the first saponification or sensitization in time, temperature and concentration such that the yarns at those places treated lose only about 2 to 7 per cent of their weight. Obviously, the concentration, temperature and duration of treatment of the yarns will vary according to the sensitizing agent employed to produce this limited degree of saponification. As this sensitizing of the yarns or fabric is preferably done during a winding operation the period of time of action and penetration is relatively short and the temperature is about room temperature, the concentration should be such that the solution applied has a pH value of above 10.

After the yarns have been sensitized as above described, that is, to such an extent that they have lost between 3 and 7 per cent of their weight, the same may be formed into cloth or fabric by any suitable method. Cloth or fabric so formed may then be treated in a developing bath or given a second treatment to saponify the places of the yarns sensitized to any desired extent. The second or developing bath preferably consists of a basic solution having a pH value of between 8 to 10.5 and the duration and temperature of treatment so regulated that the unsensitized portions of the yarn, if any, are unaffected by the second treatment. The preferable method of carrying out this second step of saponification is to treat the fabric in a bath containing from 5 to 10 grams per litre or more of soap in an aqueous media at a temperature from 70° C. to boiling. The duration of treatment in the soap bath will depend upon the sensitization, the soap and the temperature of the bath and may vary between 10 minutes and one hour, depending upon the degree of saponification desired. Although soap solutions are normally preferred for developing and further saponifying the sensitized yarns, any basic solution having a pH value between 8 and 10.5 may be employed and for this purpose dilute solutions of the reagents named above as sensi-

tizing agents may be employed. By varying the concentration, the time and temperature of the developing or second saponifying bath, the sensitized parts of the yarn or fabrics may be caused to lose as much as 20 per cent or more of their weight without any appreciable saponification being apparent on the unsensitized portion of the yarn or fabric. <sup>10</sup> The sensitized or periodically sensitized yarn produced by partially saponifying over intermittent lengths of the yarn during the winding operation may be further saponified in after treatments of the yarn or fabric produced therefrom; such further saponification affecting only the saponified or sensitized places with substantially no saponification taking place on the unsaponified or unsensitized places. This further saponification or second saponification may be desired to obtain greater depth in shade than where only a light periodic saponification has been applied originally, or even to obtain such a degree of saponification that the saponified places substantially or completely resist dyestuffs which normally dye cellulose acetate and like yarns but which have no affinity for cotton and the regenerated cellulose yarns. This further saponification or development may be effected by treating the yarns or fabrics in hydrolyzing baths of moderate pH value such as, for example, 9 or 10, which normally have substantially no hydrolyzing or very little and slow hydrolyzing action on the yarns containing organic esters of cellulose. <sup>20</sup>

These baths may consist of, for example, soap and water, sodium acetate and water, and various buffered baths containing sodium, potassium or other similarly reacting salts in the presence of buffering substances or without the aid of such buffering substances. The result of the immersion in such baths is to increase the saponification in the saponified or sensitized places with substantially no saponification in the unsaponified or unsensitized places and the result of the reaction is more rapid when the temperature of the bath is elevated, for example, to 80° C. up to the boil. The increase in saponification is appreciable in such baths even within such times as 10 to 30 minutes. <sup>30</sup>

If it is not desired to increase the saponification of yarns or fabrics sensitized in accordance with this invention and it is desirable to treat the goods in soap and similarly reacting baths, then the goods may be pretreated by washing the reaction product of sensitizing material with the yarn away from the fabric first with water which removes the acetate or other salt of the base formed on the yarn or fabric during the sensitizing operation. Also, the subsequent saponification of the yarn when treated in soap baths, etc. may be prevented by washing in dilute acids prior to entering the scouring bath containing the soap. By thus treating the yarn either by washing or by a treatment in a dilute acid the whole of the yarn is brought to such a state that any saponification treatment applied thereto will not affect the previously sensitized or saponified portions more than the unsensitized or unsaponified portions. <sup>40</sup>

As an aid to illustrating this invention and not as limitations, the following examples are given:

#### Example I

An acetone soluble cellulose acetate yarn is placed in a humidor having an atmosphere of relative humidity above 65 per cent for such a period of time that the moisture regain of the

yarn amounts to about 4 per cent on the weight of the yarn. The yarn is placed on the supply bobbin spindle of a re-winding machine and wound at 100 meters per minute and caused to contact with a furnishing roller or other device applying a 20 per cent solution of sodium hydroxide to the yarn in such an amount that the yarn is saponified to a weight loss of 5 per cent when the yarn is washed in cold water to remove the sodium acetate formed and its weight loss determined. A quantity of this yarn not washed in cold water is treated in 10 grams per litre soap solution at 99° C. for 30 minutes. It is found that the saponification has progressed to a weight loss of 10 per cent and the affinity for cotton colors correspondingly increased. It is found that the saponification of the yarn is uniform throughout its length and woven into a fabric and dyed shows substantially no unevenness due to irregularities in the depth or amount of saponification of the yarn.

*Example II*

Example I is repeated except that the yarn during the winding operation is caused to periodically contact with a furnishing device furnishing a sensitizing material containing a 20 per cent solution of sodium hydroxide, instead of continuously sensitizing the yarn. The yarn dyed with a cotton dyestuff is found to have a sharp line between the part of the yarn having an affinity for the cotton dyestuff and the unsaponified part of the yarn. The yarn at the parts thereof that have been saponified are found to take dyes having affinity for cotton evenly, without streaks or variations in shade.

*Example III*

A fabric is formed from yarns containing an acetone soluble cellulose acetate, which fabric is rolled into a package. The fabric is placed in a chamber having an atmosphere of relative humidity above 65 per cent for a period of time such that the moisture regain of the yarn amounts to about 4 per cent on the weight of the yarn. The fabric is passed through a printing device that applies to the fabric in a pattern a paste containing a saponifying agent. The fabric is then treated in a heated bath containing 10 grams per litre of soap for 20 minutes. The pattern is found to be developed and takes dyes having affinity for cotton.

While in the foregoing specification I have cited specific instances and examples, it is not my intention that the scope of the invention should be limited thereby as many modifications in this process may be employed without departing from the spirit of my invention.

Numerous effects may be obtained on the yarn or fabrics produced therefrom by applying to various portions of the yarn a varying amount of sensitizing material which results when developing the yarn in a soap bath in a yarn having portions, each portion having a correspondingly different degree of saponification and affinity for the various dyestuffs. Further, there may be produced novel effects on the yarn or fabric in two winding operations, the material having a different moisture content in each winding operation, thus varying the amount and type of sensitizing places on the material.

The yarns prior to being treated in an atmosphere having a relatively high humidity may be lubricated. It is preferred when employing a lubricant for such yarns to employ one which is

non-saponifiable and one which permits a relatively fast regain of moisture content of the yarn when the same is placed in a humid atmosphere. An example of a preferred lubricant is a dispersion of sulphonated naphthene in mineral oil that may or may not contain an acid color as a tinting compound.

Having described my invention what I desire to secure by Letters Patent is:

1. Process for saponifying filaments, yarns, fabrics and other materials having a basis of ester of cellulose, which comprises subjecting the materials to the action of a humid atmosphere to increase their moisture content, and subsequently saponifying the materials while they still possess a high moisture content.

2. Process for saponifying filaments, yarns, fabrics and other materials having a basis of organic ester of cellulose, which comprises subjecting the materials to the action of a humid atmosphere to increase their moisture content, and subsequently saponifying the materials while they still possess a high moisture content.

3. Process for saponifying filaments, yarns, fabrics and other materials having a basis of cellulose acetate, which comprises subjecting the materials to the action of a humid atmosphere to increase their moisture content, and subsequently saponifying the materials while they still possess a high moisture content.

4. Process for saponifying filaments, yarns, fabrics and other materials having a basis of cellulose acetate, which comprises subjecting the materials to the action of a humid atmosphere to increase their moisture content substantially to its maximum value at the temperature of treatment, and subsequently saponifying the materials while they still possess this moisture content.

5. A process of manufacturing artificial materials, which comprises subjecting yarns, filaments, fabrics and other materials having a basis of organic ester of cellulose to the action of a humid atmosphere whereby their moisture content is raised substantially, sensitizing to saponification at least part of the materials by treatment with a solution having a basic reaction, and then subjecting them to the action of an alkaline saponifying agent.

6. A process of manufacturing artificial materials, which comprises subjecting yarns having a basis of organic ester of cellulose to the action of a humid atmosphere whereby their moisture content is raised substantially, subjecting the yarns at intervals along their length to a preliminary saponification during a winding operation, and subsequently subjecting the yarns to further saponification with a substance of low alkalinity while they still contain reaction products derived from the preliminary saponification.

7. Process for locally saponifying filaments, yarns, fabrics and other materials having a basis of organic ester of cellulose, which comprises subjecting the materials to the action of a humid atmosphere to increase their moisture content, removing from selected areas of the material a small proportion of its acetyl content by pretreatment with an alkaline saponifying agent, whereby the material wherever pretreated is rendered more sensitive to saponification, and subsequently completing the desired saponification of the pretreated areas by treating the material, while it still contains reaction products derived from the pretreatment, with an alkaline substance which is less alkaline than that employed in the pretreatment and which has substantially no saponifying

action on the areas of the material which have not been pretreated.

8. Process for locally saponifying filaments, yarns, fabrics and other materials having a basis of cellulose acetate, which comprises subjecting the materials to the action of a humid atmosphere to increase their moisture content, removing from selected areas of the material a small proportion of its acidyl content by pretreatment 10 with an alkaline saponifying agent, whereby the material wherever pretreated is rendered more sensitive to saponification, and subsequently completing the desired saponification of the pretreated areas by treating the material, while it still contains reaction products derived from the pretreatment, with a solution having a pH value of from 8 to 11 and which is less alkaline than that employed in the pretreatment and which has substantially no saponifying action on the areas of the material which have not been pretreated.

9. Process for locally saponifying filaments, yarns, fabrics and other materials having a basis of organic ester of cellulose, which comprises subjecting the materials to the action of a humid atmosphere to increase their moisture content, removing from selected areas of the material a small proportion of its acidyl content by pretreatment with a saponifying solution having a pH value of from 10 to 14, whereby the material wherever pretreated is rendered more sensitive to saponification, and subsequently completing the desired saponification of the pretreated areas by treating the material, while it still contains reaction products derived from the pretreatment, 30 with a solution having a pH value of from 8 to 11 and which is less alkaline than that employed in the pretreatment and which has substantially no saponifying action on the areas of the material which have not been pretreated.

10. Process for locally saponifying filaments, yarns, fabrics and other materials having a basis of cellulose acetate, which comprises subjecting the materials to the action of a humid atmosphere to increase their moisture content, removing from selected areas of the material a small proportion of its acidyl content by pretreatment 40 with a saponifying solution having a pH value of from 10 to 14, whereby the material wherever

pretreated is rendered more sensitive to saponification, and subsequently completing the desired saponification of the pretreated areas by treating the material, while it still contains reaction products derived from the pretreatment, with a solution having a pH value of from 8 to 11 and which is less alkaline than that employed in the pretreatment and which has substantially no saponifying action on the areas of the material which have not been pretreated.

5

11. Process for locally saponifying artificial materials having a basis of cellulose acetate, which comprises subjecting the materials to the action of a humid atmosphere to increase their moisture content, removing from selected areas of the material during a winding operation a small proportion of acidyl content by pretreatment 15 with an alkaline saponifying agent, whereby the material wherever pretreated is rendered more sensitive to saponification, and subsequently 20 completing the desired saponification of the pretreated areas by treating the material, while it still contains reaction products derived from the pretreatment, with an alkaline substance which is less alkaline than that employed in the pretreatment and which has substantially no saponifying 25 action on the areas of the material which have not been pretreated.

12. Process for locally saponifying artificial materials having a basis of cellulose acetate, 30 which comprises subjecting the materials to the action of a humid atmosphere whereby their moisture content is raised substantially to its maximum value at the temperature of treatment, removing from selected areas of the material a small proportion of its acidyl content by pretreatment 35 with an alkaline saponifying agent, whereby the material wherever pretreated is rendered more sensitive to saponification, and subsequently completing the desired saponification of the pretreated areas by treating the material, while it still contains reaction products derived from the pretreatment, with an alkaline substance which is less alkaline than that employed in the pretreatment and which has substantially no saponifying 40 action on the areas of the material which have not been pretreated.

45 WILLIAM WHITEHEAD.